

## UNITED STATES PATENT OFFICE

2,029,724

NITRIDED STEEL AND A PROCESS FOR ITS  
PRODUCTION

Wilhelm Kroll, Luxemburg, Luxemburg

No Drawing. Application January 6, 1931, Serial  
No. 506,973. In Germany January 18, 1930

14 Claims. (Cl. 148—16)

The invention relates to nitrided steel and a process for its production.

It is already known that iron as well as certain alloyed steels can be superficially nitrided by heating in a current of ammonia at temperatures between 500° and 800° C. (nitriding). In particular chrome-aluminium steels are nitrided at a temperature below 580° at which there is still produced no coating tending to form splinters.

10 The invention relates to the use of beryllium-containing steels such as nitrided steels and to a process for the nitriding of these steels. By means of experiments it has been found that beryllium-nitrided steels possess great technical advantages.

15 As is well known beryllium steels, in particular those alloyed with nickel, also chrome-containing beryllium steels will age if after chilling from a higher range of temperature they are subjected 20 to the so-called artificial ageing, that is to say to a subsequent heat treatment at temperatures between about 400 to 600° C. The chilled beryllium steels by such ageing process attain their great hardness at those temperatures at which 25 nitriding is conducted. Consequently according to the invention it is possible by nitriding to coat a beryllium steel which in the aged state has a hardness of 600-700 Brinell, with a coating as hard as glass, which is impossible with the ordinary chilled steels because the steel is already 30 annealed by the nitriding temperatures. By the use of my invention I can produce a metal body or article which possesses a core as hard as steel and a surface as hard as glass. As, furthermore, 35 beryllium has a rather considerable affinity for nitrogen the carrying out of the nitriding process is facilitated and generally speaking the work can be done with nitriding temperatures of 500° C.

40 It is possible by a single operation, to age beryllium steels artificially and, at the same time to nitride them. If desired, however, the nitriding can be effected after the artificial ageing of the beryllium steels.

45 It has been found that the best results are obtained when the percentage of beryllium is between 0.1 and 5%. In some cases somewhat more or somewhat less beryllium can be used. Especially favourable properties are exhibited by a 50 nitrided steel with 10-12% nickel, say with about just as much chromium and 1% beryllium. The percentage of chromium may if desired be increased to over 20%. Invar-steels are also capable of being nitrided provided they contain 55 beryllium.

It is well-known that invar-steels contain about 36% of nickel.

I claim:

1. As a new article of manufacture, a steel having a nitrided surface layer and containing from .1 to 5% of beryllium, the principal portion of the remainder being iron. 5

2. As a new article of manufacture, a steel having a nitrided surface layer and containing from .1 to 5% of beryllium, and about from 10 to 12% 10 of nickel, the principal portion of the remainder being iron.

3. As a new article of manufacture, a steel having a nitrided surface layer and containing from .1 to 5% of beryllium, about from 10 to 12% of 15 nickel and about from 10 to 20% of chromium, the principal portion of the remainder being iron.

4. As a new article of manufacture, a steel chilled from a temperature above that of aging and subsequently heated in an atmosphere containing nitrogen to a temperature of from 400 20 to 600° C. until nitrogen has penetrated into its surface to form a nitrided layer, said steel containing from .1 to 5% of beryllium, the principal portion 25 of the remainder being iron.

5. As a new article of manufacture, a steel chilled from a temperature above that of aging and subsequently heated in an atmosphere containing nitrogen to a temperature of from 400 to 600° C. until nitrogen has penetrated into its 30 surface to form a nitrided layer, said steel containing from .1 to 5% of beryllium and about from 10 to 12% of nickel, the principal portion of the remainder being iron.

6. As a new article of manufacture, a steel chilled from a temperature above that of aging and subsequently heated in an atmosphere containing nitrogen to a temperature of from 400 to 600° C. until nitrogen has penetrated into its 35 surface to form a nitrided layer, said steel containing from .1 to 5% of beryllium, about from 10 to 12% of nickel and about from 10 to 20% of chromium, the principal portion of the remainder being iron. 40

7. The process of improving the hardness of steel containing from .1 to 5% of beryllium, the principal portion of the remainder being iron, which process consists in chilling the steel from a temperature above that of aging and subsequently nitriding it superficially while heating it 50 to a temperature of from 400 to 600° C.

8. The process of improving the hardness of steel containing from .1 to 5% of beryllium and about from 10 to 12% of nickel, the principal portion of the remainder being iron, which proc- 55

ess consists in chilling the steel from a temperature above that of aging and subsequently nitriding it superficially while heating it to a temperature of from 400 to 600° C.

- 5 9. The process of improving the hardness of steel containing from .1 to 5% of beryllium, about from 10 to 12% of nickel and about from 10 to 20% of chromium, the principal portion of the remainder being iron, which process consists in
- 10 chilling the steel from a temperature above that of aging and subsequently nitriding it superficially while heating it to a temperature of from 400 to 600° C. to produce a nitrided surface.
10. As a new article of manufacture, a steel 15 having a nitrided surface layer and containing from .1 to 5% of beryllium, and about 36% of nickel, the principal portion of the remainder being iron.
11. As a new article of manufacture, a steel 20 chilled from a temperature above that of aging and subsequently heated in an atmosphere containing nitrogen to a temperature of from 400 to 600° C. until nitrogen has penetrated into its

surface to form a nitrided layer, said steel containing from .1 to 5% of beryllium and about 36% of nickel, the principal portion of the remainder being iron.

12. The process of improving the hardness of steel containing from .1 to 5% of beryllium and about 36% of nickel, the principal portion of the remainder being iron, which process consists in chilling the steel from a temperature above that of aging and subsequently nitriding it superficially while heating it to a temperature of from 400 to 600° C.

13. As a new article of manufacture, a nickel-alloy steel having a nitrided surface layer and containing from .1 to 5% of beryllium, the principal portion of the remainder being iron.

14. As a new article of manufacture, a nickel-chromium-alloy steel having a nitrided surface layer and containing from .1 to 5% of beryllium, the principal portion of the remainder being iron.

WILHELM KROLL.